

O. Marland,

2. Sheets. Sheet 1.

Safe.

No. 101,824.

Patented Apr. 12. 1870.

Fig. 1.



Fig. 2.



Witnesses { W. B. Bushy  
(Francis Smith

Obadiah Marland

O. Marland,

2 Sheets, Sheet 2.

Stage.

No. 101,824.

Patented Apr. 12, 1870.

Fig. 3.



Fig. 4.



Fig. 5

Fig. 6.



Witnesses { W. B. Crosby  
Francis Gould

Obadiah Marland

# United States Patent Office.

OBADIAH MARLAND, OF BOSTON, MASSACHUSETTS.

Letters Patent No. 101,894, dated April 12, 1870.

## IMPROVEMENT IN SAFES.

The Schedule referred to in these Letters Patent and making part of the same.

To all whom it may concern:

Be it known that I, OBADIAH MARLAND, of Boston, in the county of Suffolk and State of Massachusetts, have invented Improvements in Safes; and I do hereby declare that the following, taken in connection with the drawings which accompany and form part of this specification, is a description of my invention sufficient to enable those skilled in the art to practice it.

In the patent No. 77,432 issued for my invention April 28, 1868, I describe safes, the top, bottom, sides, and door of which are each made of or with one plate, which is composed of layers of iron and steel, welded together and hardened.

My present improvement consists in a safe in which the sides, top, and bottom are formed of one continuous band of united layers of iron and steel, whether welded together or made of one homogeneous piece and then converted, in which band the steel is hardened instead of being formed of four separate plates, as in my patent before referred to, said continuity of structure saving four joints at the corners or angles of the safe, and adding greatly to the strength thereof; and

My said improvement further consists in a safe which has either the top, bottom, sides, back, door, and door-frame; and preferably all of them, each made of or with a single piece, which is first either all iron or steel, and is then changed by conversion into layers of iron and steel, which are integral and blend one into the other, each piece having always two or three layers, but generally and preferably three, of which one layer at least is always steel, the steel layer or layers being hardened in each piece after it is fitted in all respects to shape and for attachments, and before it is finally united with the others to make a safe.

In the drawings illustrating an embodiment of my invention—

Figure 1 is a vertical cross-section of a safe, showing the sides, top, and bottom, as made in a band or belt, without a seam, and of combined layers of iron and steel.

Figure 2 is a vertical section, taken in a plane extending from front to rear of a safe, and exhibiting the joints of the back and door-frame with the top and bottom, the joints of the back and door-frame with the sides, and the joints of the sides with the top and bottom being like those first mentioned. Said figure also shows how said parts are held together by screws *b*, which pass through angle-irons *a*, placed within the safe at the angles or corners, into the said parts in which the screw-holes are bored, but only partly through the thickness of said parts, and are tapped with nut-threads. The screws are preferably made of mingled iron and steel, and the steel hardened.

Figure 3 is a sectional elevation of the door-frame. Figure 4 is a sectional elevation of the back or rear plate of the safe.

Figure 5 is a sectional elevation of a safe or vault-door.

In the drawings the short close hatch lines are intended to denote where the material is changed for conversion. For example, if the plate is of iron and then packed in carbon and submitted to a sufficient degree of heat a sufficient time, the outer parts of the plate shown by the short close hatch lines will become carbonized or stealed, and may be hardened by any of the usual processes of hardening steel. If the plate is of steel, and is then packed in oxide of iron and submitted to a sufficient degree of heat a sufficient time, the outer parts of the plate represented by the short close hatch lines will lose their carbon and be reduced to soft iron which will not be hardened by the processes that will harden the steel surrounded by the iron. Or the steel may be superficially decarbonized in any other known way.

If the iron or steel plates are packed on but one surface with carbon or oxide respectively, then the result will be plates of but two layers, one of iron and one of steel. And where in the drawings the short close hatch lines are to be understood as representing steel, the longer hatch lines, which are at greater distances apart, are to be understood as representing iron, and *vice versa*.

The plates for the top, bottom, sides, and back, and the door-frame, are made and are converted and fitted together, the door-frame being also fitted to receive the rebates of the door, and the bolts, dogs, and hinges thereon. Then the parts are hardened, and if warped or sprung are brought back into place by any suitable means, the soft iron in the parts retaining the impression given and preventing the steel from springing back.

The door-frame, when made of proper size, is converted and wrought to fit the safe walls and door, and provided with hinges, and hardened, corrected, and secured in place.

The door is made of one plate, brought to the right size, converted, and then wrought on all its edges to fit the rebates in the door-frame, and with hinges, dogs, and provision to receive the lock, bolts, and handle, after which it is hardened and corrected and adjusted in place.

To make the top, bottom, and sides in but one piece, I take a plate of proper size and bend it with suitable rounded corners or with sharp angles, as may be preferable, so as to make the ends of the plate (suitably formed or scarf'd) come together, and then weld them into a band. If the plate or band so formed is not made of layers of iron and steel welded

together in strata, then I convert it in the manner in which I have explained that I convert the sides, top, bottom, back, and door-frame.

After this, I work in the edges of the band the rebates to receive the back and door-frame, or the door if no frame is used, and having made the screw-holes and other necessary fittings in and on the band, I harden its steel and then correct its form, and apply and fix in place the back and door-frame and door.

The safe described is supposed to be burglar-proof, and it may receive additions to make it fire-proof by inclosing it within suitable walls of iron or masonry containing non-conductors, and water in suitable vessels may be placed in the walls of the non-conducting material, or within the space of the burglar-proof safe, to be evaporated by and to absorb and carry off the heat penetrating to the interior.

The making of the rebates for the joints may be done before the metal is converted, in which case the conversion will be at the joints, as represented in the drawings before mentioned; but if the conversion is effected when the plates are brought to size merely, and then the rebates are afterward made, the condition of the metal will be as shown in Figure 6, on a scale larger than the other figures.

For reasons obvious to safe-makers, I prefer to con-

vert the outside of steel plates into iron rather than to convert the outside of iron plates into steel.

I claim—

A safe or chest, any single boundary of which is protected by one plate, of such size that there shall be no joint through said boundary, when such plate is made of iron or steel changed superficially by conversion, and in which the steel is hardened, substantially as described.

Also, a door-frame for a safe, vault, or chest, when said frame is made in one integral piece of soft iron and hard steel, substantially as described.

Also, a safe or chest or vault-door, made of or protected by a plate covering the entire opening which the door controls, when said plate is made of iron or steel superficially changed by conversion, and in which the steel is hardened, substantially as described.

Also, a safe or chest, the sides, top, and bottom of which are made of strata of combined iron and steel as a continuous band without joints, and in which the steel is hardened.

OBADIAH MARLAND.

Witnesses:

J. B. CROSBY,  
FRANCIS GOULD.